

## UNITED STATES PATENT OFFICE.

RICHARD METZGER, OF HEIDELBERG, GERMANY, ASSIGNOR TO I. G. FARBEIN-DUSTRIE AKTIENGESELLSCHAFT, OF FRANKFORT-ON-THE-MAIN, GERMANY, A CORPORATION OF GERMANY.

## DYEING AND PRINTING CELLULOSE ESTERS.

No Drawing. Application filed March 4, 1926, Serial No. 92,345, and in Germany March 6, 1925.

I have found that water-soluble sulfamic acids derived from colored amino compounds which are not dyestuffs in a usual sense, especially from amino-anthraquinones, are excellently suitable for dyeing and printing cellulose esters and fabrics made thereof. These sulfamic acids can be used as such or in the state of salts and may contain one or several  $\text{NH}-\text{SO}_3\text{H}$  residues with or without further substituents in their molecules.

The dyeing process may be carried out in the usual manner without any preliminary treatment of the cellulose ester as for example a partial saponification thereof being necessary. In many cases the dyeings so obtained may be subjected to an after-treatment with diazo compounds or they may be diazotized and coupled with a suitable component, by which after-treatments valuable new shades are obtained. The printing may also be carried out in the usual manner and bright beautiful shades are obtained thereby.

The following examples will further illustrate the manner of carrying the invention out in practice, to which examples, however, the invention is not limited. The parts are by weight.

## Example 1.

Cellulose acetate silk is introduced into a luke-warm dyebath prepared by dissolving 3 per cent of the sulfamic acid sodium salt derived from 1,4-diamino-anthraquinone (of 30 per cent purity) in warm water and adding to this solution 10 per cent of Glauber's salt and 4 per cent of sulfuric acid (all quantities are calculated on the weight of the cellulose acetate). The temperature is slowly raised to 70 degrees to 80 degrees centigrade. A beautiful reddish violet dyeing is obtained. Instead of sulfuric acid a greater quantity of formic acid may be employed, whereby somewhat lighter shades are obtained.

## Example 2.

Cellulose acetate silk is dyed beautiful red-

dish blue shades at about 75 degrees centigrade from a dye-bath prepared by dissolving 3 per cent of the sodium salt of 1,5-disulfamic acid-4,8-dihydroxy-anthraquinone (of about 54 per cent purity) in water and adding 10 per cent of sodium bisulfate in one or several portions.

## Example 3.

50 parts of the sulfamic acid sodium salt derived from 1-amino-4-methoxy-anthraquinone (of 43 per cent purity) are dissolved in 50 parts of glycerol and made into a paste by means of 900 parts of a thickening mixture. Cellulose acetate silk is printed with this paste, dried, steamed and rinsed. The silk is colored bright bluish red shades.

What I claim is:—

1. The process of dyeing and printing cellulose esters which consists in applying to the goods a water-soluble sulfamic acid derived from a coloured amino compound which is not a dyestuff of itself.

2. The process of dyeing and printing cellulose esters which consists in applying to the goods a water-soluble sulfamic acid derived from an amino-anthraquinone.

3. The process of dyeing and printing cellulose esters which consists in applying to the goods a water-soluble sulfamic acid derived from a coloured amino compound which is not a dyestuff, and diazotizing the dyeing and combining it with a suitable dyestuff component.

4. The process of dyeing and printing cellulose esters which consists in applying to the goods a water-soluble sulfamic acid derived from an amino-anthraquinone which is not a dyestuff, diazotizing the compound applied to the goods and coupling it with an azo dyestuff component.

In testimony whereof I have hereunto set my hand.

RICHARD METZGER.